

# United States Patent Office

2,973,388

Patented Feb. 28, 1961

1

2,973,388

## ALIPHATIC POLYETHERS

Randolph Riemschneider, Berlin-Charlottenburg, Germany, assignor to Ethyl Corporation, New York, N.Y., a corporation of Delaware

No Drawing. Filed July 31, 1957, Ser. No. 675,254

3 Claims. (Cl. 260—615)

This invention relates to synthetic lubricating compositions. More particularly, this invention relates to synthetic lubricants having superior performance characteristics, especially outstanding resistance to oxidative deterioration.

The large number of materials used as lubricants shows that the many different purposes of lubricant application require the choice, in each case according to the particular lubricating requirements and operating conditions, of materials which fulfill as many of the requirements as possible. However, this is not always possible. Some lubricants are not stable enough toward oxidants, corrosion, and heating; others have too low a lubricant strength and too little lubricity or cannot withstand extreme pressures. Oftentimes small amounts of one or more additives compensate for these deficiencies. Also, the use of completely different classes of materials have been investigated, e.g., silicones, instead of lubricating oils obtained from petroleum fractions or instead of synthetic oils based on hydrocarbons or esters. The search continues for materials which have not yet been used for lubrication but which are suitable therefor and which can fill certain gaps in the previous choice of lubricants.

An object of this invention is to provide novel and highly useful synthetic lubricants. Another object is to provide synthetic lubricating compositions characterized by outstanding stability against oxidation. Another object is to provide new compositions of matter. A further object is to provide methods of effectively lubricating relatively-moving metallic surfaces which are normally in contact with each other. Other objects will be clear from the following description of this invention.

The present invention comprises essentially the use of ethers as lubricants, particularly those organic compounds which contain several R—O—R' linkages, wherein R and R' signify the same or different hydrocarbon radicals. It should be understood that for the purposes of lubrication, only those ethers are to be considered which have high enough boiling points so that they are practically non-volatile at the usual temperature and which have an oily nature or which are solid, plasticizable substances.

It has been shown that ethers of the aforesaid type are not only equivalent to the previously known lubricants but are even superior in many respects.

Particularly useful as synthetic lubricants are ethers having a total of 10 to 27 carbon atoms in the molecule and a boiling point at atmospheric pressure of at least 180° C., the ethers being represented by the following formulas:

(1)  $R_1—O—R_2$

wherein R<sub>1</sub> contains 1 to 6 carbon atoms and is selected from the group consisting of alkyl, alkenyl and cycloalkyl groups and R<sub>2</sub> contains 10 to 16 carbon atoms and is

2

selected from the group consisting of branched chain alkyl and branched chain alkenyl groups;

(2)  $R_3—O—R_4—O—R_5$

5 wherein R<sub>3</sub> contains 1 to 12 carbon atoms and is selected from the group consisting of alkyl and cycloalkyl groups, R<sub>4</sub> is a divalent aliphatic hydrocarbon radical containing 2 to 8 carbon atoms and R<sub>5</sub> contains 2 to 18 carbon atoms and is selected from the group consisting of alkyl, alkenyl, 10 cycloalkyl, cycloalkyl-substituted alkyl and aralkyl groups;

(3)  $R_6—O—R_7—O—R_8$

wherein R<sub>6</sub> contains 1 to 7 carbon atoms and is selected from the group consisting of alkyl and cycloalkyl groups, 15 R<sub>7</sub> is an alkylene group containing 9 to 18 carbon atoms and R<sub>8</sub> contains 1 to 12 carbon atoms and is selected from the group consisting of alkyl and cycloalkyl groups;

(4)  $R_9—O—CH_2—C≡C—CH_2—O—R_{10}$

20 wherein R<sub>9</sub> and R<sub>10</sub> are alkyl groups containing 4 to 10 carbon atoms;



25 wherein R<sub>11</sub> and R<sub>12</sub> are alkyl groups containing 4 to 10 carbon atoms;

(6)  $R_{13}—O—C_2H_4—O—C_2H_4—O—R_{14}$

wherein R<sub>13</sub> is an alkyl and aralkyl group containing 3 to 10 carbon atoms and R<sub>14</sub> contains 5 to 20 carbon atoms 30 and is selected from the group consisting of alkyl, cycloalkyl and aralkyl groups;

(7)  $R_{15}—O—C_2H_4—O—C_2H_4—O—C_2H_4—O—R_{16}$

wherein R<sub>15</sub> contains 3 to 8 carbon atoms and is selected 35 from the group consisting of alkyl and cycloalkyl-substituted alkyl groups and R<sub>16</sub> contains 5 to 16 carbon atoms and is selected from the group consisting of alkyl, cycloalkyl and aralkyl groups;



40 wherein each R<sub>17</sub> is an alkyl group containing 2 to 5 carbon atoms and R<sub>18</sub> contains 6 to 10 carbon atoms and is selected from the group consisting of alkyl and alkenyl groups;



45 wherein R<sub>19</sub> is an alkyl group containing 1 to 3 carbon atoms, R<sub>20</sub> contains 3 to 8 carbon atoms and is selected from the group consisting of alkyl and aralkyl groups and R<sub>21</sub> contains 3 to 8 carbon atoms and is selected from the group consisting of alkenyl and aralkyl groups;



50 wherein R<sub>22</sub>, R<sub>23</sub> and R<sub>24</sub> are alkyl groups containing 1 to 4 carbon atoms;



wherein  $R_{25}$ ,  $R_{26}$ ,  $R_{27}$  and  $R_{28}$  are alkyl groups containing 1 to 4 carbon atoms.

Many of the above ethers are new compositions of matter. Of these, especially good results are achieved by the use, as synthetic lubricants, of the ethers designated above as (4)-(11) inclusive, particularly when  $R_{14}$  is different from  $R_{13}$  and the total number of carbon atoms in  $R_{13}$  and  $R_{14}$  is from 8 to 21 and when  $R_{16}$  is different from  $R_{15}$  and the total number of carbon atoms in  $R_{15}$  and  $R_{16}$  is from 8 to 19.

According to the invention, the ethers cited in the following table are very useful lubricants. They are given only as examples and, therefore, do not limit the scope of the invention.

|    |                                                                                                                                                                                                                                                                                                                                                                                                                                                                | 4             |
|----|----------------------------------------------------------------------------------------------------------------------------------------------------------------------------------------------------------------------------------------------------------------------------------------------------------------------------------------------------------------------------------------------------------------------------------------------------------------|---------------|
|    | Isoamyl-tert-heptyl ether of pentane diols                                                                                                                                                                                                                                                                                                                                                                                                                     | 178 (7-9)     |
|    | C <sub>18</sub>                                                                                                                                                                                                                                                                                                                                                                                                                                                |               |
| 5  | Butyl-tris-propyl-ether of pentaerythritol                                                                                                                                                                                                                                                                                                                                                                                                                     | 300           |
|    | Bis-octyl-glycol ether                                                                                                                                                                                                                                                                                                                                                                                                                                         | 290           |
|    | Cyclopentyl-isoundecyl-glycol ether                                                                                                                                                                                                                                                                                                                                                                                                                            | 185 (9)       |
|    | 1,8-diaminooxy-octane                                                                                                                                                                                                                                                                                                                                                                                                                                          | 212 (30)      |
|    | Bis-benzyl-methyl-ether of glycerine                                                                                                                                                                                                                                                                                                                                                                                                                           | 255-260       |
|    | C <sub>19</sub>                                                                                                                                                                                                                                                                                                                                                                                                                                                |               |
| 10 | n-Tetradecyl-n-propyl-glycol ether                                                                                                                                                                                                                                                                                                                                                                                                                             | 184 (5)       |
|    | n-Dodecyl-n-propyl-diglycol ether                                                                                                                                                                                                                                                                                                                                                                                                                              | 170-172 (0.9) |
|    | Methyl-n-decyl-ether of 2,5-dimethyl-hexane-diol-1,3                                                                                                                                                                                                                                                                                                                                                                                                           | 186 (3-5)     |
|    | Propyl-hexyl-ether of 2-hexyl-2-methyl-propyl-diol-1,3                                                                                                                                                                                                                                                                                                                                                                                                         | 205 (25)      |
|    | Cyclopentyl-isotetradecyl-ether                                                                                                                                                                                                                                                                                                                                                                                                                                | 184-186 (4)   |
| 15 | Butyl-pentyl-ether of 2-isopropyl-4,4-dimethyl-pentane-diol-1,3                                                                                                                                                                                                                                                                                                                                                                                                | 200 (13)      |
|    | Bis-cyclopentyl-ether of nonane-diol                                                                                                                                                                                                                                                                                                                                                                                                                           | 165 (0.3)     |
|    | Benzyl-butyl-tetraglycol ether                                                                                                                                                                                                                                                                                                                                                                                                                                 | 170 (0.2-0.4) |
|    | C <sub>20</sub>                                                                                                                                                                                                                                                                                                                                                                                                                                                |               |
| 20 | [Cyclopentylethyl] - isoundecyl - glycol ether                                                                                                                                                                                                                                                                                                                                                                                                                 | 163 (0.1)     |
|    | Pentadecyl-n-propyl-ether of glycol                                                                                                                                                                                                                                                                                                                                                                                                                            | 199-201 (6)   |
|    | Dodecyl-butyl-diglycol ether                                                                                                                                                                                                                                                                                                                                                                                                                                   | 185 (0.7)     |
|    | Tridecyl-cyclopentyl-glycol ether                                                                                                                                                                                                                                                                                                                                                                                                                              | 180-181 (0.2) |
|    | Bis-cyclohexyl-ether of glycol                                                                                                                                                                                                                                                                                                                                                                                                                                 | 201-203 (7)   |
|    | [Cyclohexylmethyl]-undecyl-glycol ether                                                                                                                                                                                                                                                                                                                                                                                                                        | 320-325 (200) |
|    |                                                                                                                                                                                                                                                                                                                                                                                                                                                                | 164-165 (0.2) |
| 25 | C <sub>21</sub>                                                                                                                                                                                                                                                                                                                                                                                                                                                |               |
|    | Hexadecyl-n-propyl-glycol ether                                                                                                                                                                                                                                                                                                                                                                                                                                | 207-209 (6-7) |
|    | Dodecyl-n-propyl-triglycol ether                                                                                                                                                                                                                                                                                                                                                                                                                               | 192-195 (0.8) |
|    | Propyl-dodecyl-triglycol ether                                                                                                                                                                                                                                                                                                                                                                                                                                 | 192-194 (0.9) |
|    | Phenylcyclohexyl-propyl-triglycol ether                                                                                                                                                                                                                                                                                                                                                                                                                        | 205-208 (5-8) |
| 30 | Tetrakisbutyl-ether of pentaerythritol                                                                                                                                                                                                                                                                                                                                                                                                                         | 340-342       |
|    | Dicyclohexyl-ether of 2-ethyl-1,3-heptane-diol                                                                                                                                                                                                                                                                                                                                                                                                                 | 200 (0.9)     |
|    | Bis-methylcyclopentyl-ether of 2-methyl-octane-diol-1,3                                                                                                                                                                                                                                                                                                                                                                                                        | 210 (6)       |
|    | C <sub>22</sub>                                                                                                                                                                                                                                                                                                                                                                                                                                                |               |
| 35 | Heptylcyclopentyl - isobutyl - triglycol ether                                                                                                                                                                                                                                                                                                                                                                                                                 | 200-202 (0.5) |
|    | Cyclohexyl-isocetyl-ether                                                                                                                                                                                                                                                                                                                                                                                                                                      | 220-(3-5)     |
|    | Dodecyl-n-butyl-triglycol ether                                                                                                                                                                                                                                                                                                                                                                                                                                | 205-208 (0.6) |
|    | n-Heptadecyl-n-isopropyl-glycol ether                                                                                                                                                                                                                                                                                                                                                                                                                          | 220 (5)       |
|    | Bis-benzyl-tetraglycol ether                                                                                                                                                                                                                                                                                                                                                                                                                                   | >200 (0.3)    |
|    | C <sub>23</sub>                                                                                                                                                                                                                                                                                                                                                                                                                                                |               |
|    | Octadecyl-n-propyl-glycol ether                                                                                                                                                                                                                                                                                                                                                                                                                                | 242-243 (14)  |
|    | Tetradecyl-n-propyl-triglycol ether                                                                                                                                                                                                                                                                                                                                                                                                                            | 192-194 (0.2) |
|    | Cetyl-propyl-diglycol ether                                                                                                                                                                                                                                                                                                                                                                                                                                    | 196-198 (0.8) |
|    | Cetyl-propyl-ether of butane-diol-1,4                                                                                                                                                                                                                                                                                                                                                                                                                          | 185-187 (0.4) |
| 40 | Myristyl-propyl-triglycol ether                                                                                                                                                                                                                                                                                                                                                                                                                                | 192-193 (0.2) |
|    | Cyclopentyltridecyl - isopropyl - glycol ether                                                                                                                                                                                                                                                                                                                                                                                                                 | 180-183 (0.1) |
|    | Methyl-dodecyl-ether of 2-hexyl-2-methyl-propane-diol-1,3                                                                                                                                                                                                                                                                                                                                                                                                      | 230-233 (8)   |
|    | Nonyl-decyl-ether of butane-diol-1,4                                                                                                                                                                                                                                                                                                                                                                                                                           | 190-192 (0.4) |
|    | C <sub>24</sub>                                                                                                                                                                                                                                                                                                                                                                                                                                                |               |
| 45 | Bis-propylether of octadecane-diol-1,18                                                                                                                                                                                                                                                                                                                                                                                                                        | 200-201 (0.1) |
|    | Tetradecyl-butyl-triglycol ether                                                                                                                                                                                                                                                                                                                                                                                                                               | 199 (0.1-0.3) |
|    | Octadecyl-butyl-glycol ether                                                                                                                                                                                                                                                                                                                                                                                                                                   | 235 (12)      |
|    | ( $\gamma$ -Cyclopentyl - propyl) - decyl - triglycol ether                                                                                                                                                                                                                                                                                                                                                                                                    | 201-202 (0.3) |
|    | C <sub>25</sub>                                                                                                                                                                                                                                                                                                                                                                                                                                                |               |
| 50 | Octadecyl-amyl-glycol ether                                                                                                                                                                                                                                                                                                                                                                                                                                    | 261 (12)      |
|    | Heptyl-cetyl-ether of 2-amyl-2-ethyl-propane-diol-1,3                                                                                                                                                                                                                                                                                                                                                                                                          | 240 (1-1.3)   |
|    | Decyl-nonyl-ether of quinol                                                                                                                                                                                                                                                                                                                                                                                                                                    | 230 (0.04)    |
|    | Propyl-cetyl-triglycol ether                                                                                                                                                                                                                                                                                                                                                                                                                                   | 210-212 (0.5) |
|    | Propyl-octadecyl-diglycol ether                                                                                                                                                                                                                                                                                                                                                                                                                                | 209-211 (0.6) |
|    | C <sub>26</sub>                                                                                                                                                                                                                                                                                                                                                                                                                                                |               |
| 60 | ( $\delta$ -Cyclopentyl - amyl) - decyl - triglycol ether                                                                                                                                                                                                                                                                                                                                                                                                      | 240 (0.2-0.5) |
|    | Octadecenyl-hexyl-glycol ether                                                                                                                                                                                                                                                                                                                                                                                                                                 | 267-270 (5)   |
|    | C <sub>27</sub>                                                                                                                                                                                                                                                                                                                                                                                                                                                |               |
| 65 | ( $\gamma$ -Cyclopentyl - hexyl) - dodecyl-ether of butane-diol-1,4                                                                                                                                                                                                                                                                                                                                                                                            | 233 (0.03)    |
| 70 | The above listed materials, among others, have been investigated with regard to their usefulness as lubricants using the usual tests, such as aging, viscosity, viscosity-temperature index, Conradson test, pour point, flash point and iodine number. Not only has the usefulness of these substances been confirmed, but also in many cases their superiority compared to known lubricants has been established. Above all, the ethers are distinguished by |               |
| 75 |                                                                                                                                                                                                                                                                                                                                                                                                                                                                |               |

substantially greater stability. They are three to fifteen times more stable than ester oils of corresponding constitution when the oxidation test of Ramsbottom is used for comparison. The viscosity latitude ( $W_p$ ) of many ethers lies between 0.8 and 3.0. The ethers can also be used in mixture with known lubricants. One can also use mixtures of ethers of different molecular weights or different molecular structure.

The viscosity and viscosity latitudes ( $W_p$ ) of some of the synthesized ethers are given in the following:

|                                                | 20° C. | 50° C. | 80° C. | $W_p$ |
|------------------------------------------------|--------|--------|--------|-------|
| Decyl-propyl-glycol ether.....                 | 4.056  | 2.248  | 1.468  | 2.11  |
| Dodecyl-propyl-glycol ether.....               | 5.646  | 2.948  | 1.858  | 1.78  |
| Tetradecyl-propyl-glycol ether.....            | 7.621  | 3.761  | 2.295  | 1.53  |
| Hexadecyl-propyl-glycol ether.....             | 10.439 | 4.881  | 2.892  | 1.26  |
| Octyl-propyl-diglycol ether.....               | 4.413  | 2.369  | 1.527  | 2.18  |
| Decyl-propyl-diglycol ether.....               | 6.065  | 3.082  | 1.912  | 1.85  |
| Dodecyl-propyl-diglycol ether.....             | 7.975  | 3.905  | 2.343  | 1.54  |
| Tetradecyl-propyl-diglycol ether.....          | 10.283 | 4.824  | 2.850  | 1.28  |
| Hexadecyl-propyl-diglycol ether.....           | 13.525 | 6.128  | 3.475  | 1.09  |
| Octyl-propyl-triglycol ether.....              | 6.779  | 3.278  | 2.008  | 1.93  |
| Dodecyl-propyl-triglycol ether.....            | 11.330 | 5.146  | 2.929  | 1.36  |
| Decyl-propyl-ether of butane-diol-1,4.....     | 6.206  | 3.116  | 1.963  | 1.77  |
| Hexadecyl-propyl-ether of butane-diol-1,4..... | 14.080 | 6.090  | 3.483  | 1.14  |
| Benzyl-propyl ether of butane-diol-1,4.....    | 4.677  | 2.408  | 1.535  | 2.42  |
| Benzyl-propyl diglycol ether.....              | 5.398  | 2.706  | 1.644  | 2.51  |
| Benzyl propyl triglycol ether.....             | 8.278  | 3.731  | 2.192  | 2.05  |

The pour points of ethers with straight hydrocarbon chains are higher than the pour points of ethers with branched hydrocarbon chains. The pour points of the benzyl propyl ethers of ethanediol, diglycol, triglycol and butanediol and the pour points of the corresponding cyclohexyl and cyclopentyl compounds all lie below  $-30^{\circ}\text{C}$ . The decyl-propyl ether and the decyl-isoamyl ether of butanediol-1,4 has a pour point below  $-20^{\circ}\text{C}$ . While n-decyl-propyl glycol ether has a pour point of  $-15^{\circ}\text{C}$ , a branched chain nonyl-isobutyl glycol ether has a pour point below  $-35^{\circ}\text{C}$ . Iso-nonyl-, isopropyl pentanediol ether and isononyl-, isopropyl pentanediol ether have pour points below  $-25^{\circ}\text{C}$ . Use has also been made of branched chain halides for reaction with alcoholates, e.g., 2,2-dimethyl-octylhalide; 10,10-dimethyl- and 10,10-diethyl-undecyl halide; 3-isopropyl-heptyl halide; 6-methyl- and 6-propyl-heptyl halide; 2-propyl pentylchloride; phenylethyl halide; cyclohexylethyl halide; cyclohexyl halide and others.

The ether oils were prepared by reacting the mono-sodium or monopotassium derivatives of diols, triols, tetraols, etc., with suitable halohydrocarbons or halogen compounds:



The resultant ether alcohols were then further reacted in the same manner until all the OH groups present were etherified, e.g.,



or



The following representative alcohols can be used: ethane-diol; diglycol; triglycol; tetraglycol; propanediol, butane-diol; terpinol; partially hydrated dicyclopentadienediol; amyldiol; 2-ethyl-2-tert-butyl-1,3-propanediol; 2-ethyl-1,3-pantanediol; 2,5-dimethyl-1,3-hexanediol; 2,4-dimethyl-1,3-propanediol; 2-methyl-1,3-octanediol; 2,2-diethyl-1,3-propanediol; 2-ethyl-1,3-heptanediol; 2-isopropyl-2-methyl-1,3-propanediol; 2-isopropyl-1,3-hexanediol; 2-tert-butyl-2-methyl-1,3-propanediol; 2-methyl-2-neopentyl-1,3-propanediol; 2-ethyl-2-isopropyl-1,3-

propanediol; 2-ethyl-1,3-hexanediol; 2-amyl-2-ethyl-1,3-propanediol; 2-isopropyl-1,3-pantanediol; 2-tert-butyl-2-isopropyl-1,3-propanediols; 2-ethyl-4-methyl-1,3-pantanediol; 2-isopropyl-4,4'-dimethyl-1,3-pantanediol; 2-hexyl-2-methyl-1,3-propanediol; pentaerythritol; 2,2,6,6-tetramethylol-cyclohexanone; 2,2,6,6-tetramethylol-cyclopentanol; pivalyl alcohol; quinitol; inositol; tetrahydroxycyclohexane; trihydroxycyclohexane; pentahydroxycyclohexane; octadiol; tetramethylol of the formula



15 Of the halohydrocarbons (containing chlorine, bromine, iodine) those which are branched chain are particularly suitable. The reaction with straight chain compounds, as shown in the examples, likewise takes place satisfactorily. Also, mixtures of halohydrocarbons react 20 very well with the alcoholates of the above mentioned alcohols.

### EXAMPLES

Within the scope of these experiments, more than 150 ethers have been synthesized and tested for their lubricating oil characteristics. One hundred and fifteen of these ethers are named above.

One series of experiments on the preparation of ethers of mono-, di- and triglycols is described in the following. 30 In similar manner, we have also prepared ethers of the other above-mentioned di-, tri-, tetra-, penta-ols, etc. The reactions of the alcoholates with branched chain halohydrocarbons, e.g., isohexylhalide instead of n-hexyl halide, proceed in a completely analogous manner.

#### (A) Octyl-propyl-glycol ether

(a) n-Propyl-glycol ether: 30 grams of sodium were dissolved in 280 grams of distilled glycol. This solution was mixed with 175 grams n-propyl bromide and refluxed until the bromide disappeared. Then, the reaction mixture was heated another one to two hours and fractionated without removing the precipitated NaBr.

Forecut: About 30 cc. of which 10 to 15 cc. is n-propyl bromide.

Main fraction: 149-156° C. = 127 g. = 86 percent of theory.

After cut: About 10 cc. B.P. 160° C.

50 Then the thermometer very rapidly rose up to the boiling point of ethylene glycol. The main fraction was fractionated once more whereby the main portion passed over at 150-152° C.

(b) n-Octyl-n-propyl-glycol ether: 5.1 grams of 55 sodium (smallest pieces possible) were dissolved in a mixture of 100 cc. absolute ether and 23.5 grams n-propyl glycol ether. The solution was mixed with 43 grams of octyl bromide, the ether was distilled off and the reaction mixture heated on a water bath for about one hour. The precipitated NaBr was filtered off and the filtrate fractionated in vacuum. The forecut distilled at 56-57° C./16 mm. and consisted of n-propyl glycol ether. The main fraction boiled at 132-133° C./16 mm. Yield: 80 percent of theory.



Calculated: 72.2 C; 13.05 H.

Found: 71.9 C; 13.13 H.

70 Viscosities (in centistokes):

2.914 at 20° C.

1.707 at 50° C.

1.138 at 80° C.

Pour Point: Below  $-35^{\circ}\text{C}$ .

75 Wp: 2.67.

(B) In the corresponding manner, the following reactions were also carried out:

Forecut: To 180° C./14 mm. (small amount—octyl bromide)

| No.                    | Ether Synthesized                  | Na, g. | Ether, cc. | Propylene glycol ether, g. | Halohydrocarbon           | B.P., °C.   |
|------------------------|------------------------------------|--------|------------|----------------------------|---------------------------|-------------|
| 1                      | n-Decyl-n-propyl glycol ether      | 4.5    | 100        | 20.5                       | 43.5 g. n-decylbromide    | 159-160/16  |
| 2                      | n-Dodecyl-n-propyl glycol ether    | 4.5    | 100        | 20.5                       | 49 g. dodecylbromide      | 182-184/16  |
| 3                      | n-Tetradecyl-n-propyl glycol ether | 4.5    | 100        | 20.5                       | 54.3 g. tetradecylbromide | 184-186/5   |
| 4                      | n-Hexadecyl-n-propyl glycol ether  | 4.0    | 100        | 19.0                       | 53.0 g. cetyl bromide     | 207-209/7   |
| 5                      | n-Octadecyl-n-propyl glycol ether  | 3.1    | 100        | 14.5                       | 44.5 g. octadecylbromide  | 241-243/14  |
| 6                      | Benzyl-n-propyl glycol ether       | 5.1    | 150        | 23.5                       | 29.0 g. benzyl chloride   | 135-136/16  |
| Propyl-di-glycol ether |                                    |        |            |                            |                           |             |
| 7                      | n-Octyl-n-propyl diglycol ether    | 4      | 150        | 29                         | 33 g. n-octylbromide      | 169-172/17  |
| 8                      | n-Decyl-n-propyl diglycol ether    | 4      | 150        | 29                         | 38 g. n-decylbromide      | 186-188/13  |
| 9                      | n-Dodecyl-n-propyl diglycol ether  | 4      | 150        | 29                         | 43 g. n-dodecylbromide    | 171-173/0.9 |

The monopropyl diglycol ether was prepared in the following way: 10 grams of sodium were dissolved in 160 grams of diglycol. The brown colored reaction product was cooled and mixed with 53.5 grams of n-propyl bromide. The reaction mixture was refluxed on a water bath for three hours, whereby NaBr started to precipitate out after 15 minutes. After cooling, the reaction product was mixed with somewhat more water than required for solution of the NaBr and the mixture extracted 6-7 times with ether. The ether solution was dried with  $\text{Na}_2\text{SO}_4$ , the ether evaporated off and the remainder distilled in vacuum.

Fraction 1: To 100° C./18 (small amount, odor of n-propyl glycol ether)

Main fraction: B.P.=148-150° C./0.6 mm.  
Yield: 65 percent of theory.

25  $\text{C}_{17}\text{H}_{36}\text{O}_4$  (304.46):  
Calculated: 67.05 C; 11.92 H.  
Found: 66.98 C; 11.88 H.

Viscosities (in centistokes):  
6.779 at 20° C.

30 3.278 at 50° C.  
2.008 at 80° C.

Pour point: Below -25° C.  
Wp: 1.93.

35 The following compounds were obtained under the same conditions as the octyl propyl triglycol ether:

| Ether Synthesized                     | Na, g. | Ether (cc.) | Propyl triglycol ether | Halohydrocarbon             | B.P. (°C.)  |
|---------------------------------------|--------|-------------|------------------------|-----------------------------|-------------|
| n-Dodecyl-n-propyl-triglycol ether    | 3.5    | 100         | 32                     | n-Dodecylbromide, 36 g.     | 192-194/0.9 |
| n-Tetradecyl-n-propyl-triglycol ether | 3.5    | 100         | 32                     | n-Tetradecyl bromide, 40 g. | 192-194/0.2 |

Fraction 2: 100-110° C./18 (45.5 g.=67.5 percent of theory)

Fraction 3: 128-130° C./18 (small amount, insoluble in water, soluble in ether/diglycol).

The redistilled mono-n-propyl diglycol ether boiled at 105-107° C./18 mm. Mono-n-propyl-triglycol ether: Prepared under the same conditions as n-propyl diglycol ether. From 315 grams of triglycol, 20 grams of sodium and 110 grams of n-propyl bromide, 127 grams of crude product was obtained after the ether was distilled off. Yield: 75 percent of theory. B.P.<sub>17</sub>: 148-150° C.

(C) *n-Octyl-n-propyl-triglycol ether*

In the preparation of the diether of triglycol, the product must be worked up somewhat differently, since the NaBr can be filtered off only with large losses due to the high viscosity of the ether.

3.5 grams of sodium (smallest pieces possible) were dissolved in a mixture of 100 cc. of ether and 32 grams of mono-n-propyl-triglycol ether. This was mixed with 29 grams of n-octylbromide, the ether was distilled off and the reaction mixture heated for one to two hours on a boiling water bath. After cooling, the precipitated NaBr was dissolved with about 100 cc. of water and the water-insoluble portion taken up with ether. The mixture was separated in a separatory funnel and the ether solution dried with  $\text{Na}_2\text{SO}_4$ . After evaporation of the ether, the remainder was fractionated in vacuum.

50 Besides obtaining very effective lubrication by using the foregoing ethers to lubricate relatively-moving, contacting metallic surfaces, excellent lubrication is also achieved when these ethers are used in conjunction with known lubricants. Thus, the synthetic lubricants of this invention comprise the above defined ethers, which may be used in combination with one or more standard lubricants, such as mineral lubricating oils, synthetic ester lubricants, silicones, chlorodiphenyl oils, and the like.

55 When used in these combinations, the ether preferably predominates—i.e., is present in the resultant composition in amount greater than 50 percent. However, benefits are 60 achieved by blending one or more of the above ethers with standard lubricants even at concentrations as low as 5 percent or less.

As further examples of this invention, use is made of the standard Lauson engine test. According to this test, 65 a standard spark-ignition internal combustion engine is operated for 25 hours using a standard fuel. The engine is examined before and after the test and the merit ratings as to varnish formation are given according to the test standards. The rating scale involves numbers 70 from 0 to 10, 0 being a perfect rating. Thus, this test very effectively evaluates the usefulness of the engine lubricant subjected to the test. As a baseline, the engine is operated using a highly-refined mineral lubricating oil having a viscosity of 60 Saybolt Universal Seconds at 75 210° F. as lubricant. The test is then repeated a number

of times, in each test use being made of one of the following ethers as lubricant—decyl-propyl-glycol ether; dodecyl-propyl-glycol ether; tetradecyl-propyl-glycol ether; hexadecyl-propyl-glycol ether; octyl-propyl-diglycol ether; decyl-propyl-diglycol ether; dodecyl-propyl-diglycol ether; tetradecyl-propyl-diglycol ether; hexadecyl-propyl-diglycol ether; octyl-propyl-triglycol ether; dodecyl-propyl-triglycol ether; decyl-propyl-ether of butane-diol-1,4; hexadecyl-propyl-ether of butane-diol-1,4; benzyl-propyl ether of butane-diol-1,4; benzyl-propyl-diglycol-ether; and benzyl-propyl-triglycol ether. In each instance, the use of these ethers results in superior merit ratings as compared with the baseline value.

Typical formulations provided by this invention are given in the following examples in which all percentages are by weight.

#### EXAMPLE 1

A lubricant is formulated to contain 10 percent of lauryl polymethacrylate, 5 percent of tricresylphosphate and 85 percent of 1-methoxy-7-ethoxy heptane.

#### EXAMPLE 2

A lubricant is formed from 10 percent of lauryl polymethacrylate, 5 percent of tricresylphosphate, 0.5 percent of phenothiazine with the balance being propyl-cetyl-triglycol ether.

#### EXAMPLE 3

A lubricant is formulated to contain 5 percent of lauryl polymethacrylate, 3 percent of tricresylphosphate, 12 percent of highly-refined mineral lubricating oil having a viscosity of 60 Saybolt Universal Seconds at 210° F. and 80 percent of cyclopentylisotetradecyl ether.

#### EXAMPLE 4

A lubricant is made from 10 percent of lauryl polymethacrylate, 1.5 percent of tricresylphosphate, 0.5 percent of phenyl- $\alpha$ -naphthyl amine, 44 percent of di-2-ethylhexyl sebacate and 44 percent of benzyl-propyl-triglycol ether.

#### EXAMPLE 5

A lubricant is made from 6 percent of polyisobutylene, 4 percent of triphenylphosphate, 30 percent of diisooctyl azelate and 60 percent of nonyl-decyl ether of butane-diol-1,4.

#### EXAMPLE 6

A lubricant is formulated to contain 8 percent of lauryl polymethacrylate, 2 percent of tricresylphosphate, 70 percent of tetraoctyl pentaerythritate, and 20 percent of dodecyl-n-butyl-triglycol ether.

The use of the above formulations as lubricants for aircraft gas turbine engines not only provides effective lubrication, but shows that the formulations have unusually high stability under use conditions. Other formulations involving the ether lubricants of this invention will now be apparent to those skilled in the art.

I claim:

1. As synthetic lubricants, ethers having a total of 10 to 27 carbon atoms in the molecule and a boiling point

at atmospheric pressure of at least 180° C., the ethers being selected from those having the formula



wherein  $R_{22}$ ,  $R_{23}$  and  $R_{24}$  are alkyl groups containing 1 to 4 carbon atoms, and those having the formula



wherein  $R_{25}$ ,  $R_{26}$ ,  $R_{27}$  and  $R_{28}$  are alkyl groups containing 1 to 4 carbon atoms.

2. As synthetic lubricants, ethers having a total of 10 to 27 carbon atoms in the molecule and a boiling point at atmospheric pressure of at least 180° C., the ethers having the formula



wherein  $R_{22}$ ,  $R_{23}$  and  $R_{24}$  are alkyl groups containing 1 to 4 carbon atoms.

3. As synthetic lubricants, ethers having a total of 10 to 27 carbon atoms in the molecule and a boiling point at atmospheric pressure of at least 180° C., the ethers having the formula



wherein  $R_{25}$ ,  $R_{26}$ ,  $R_{27}$  and  $R_{28}$  are alkyl groups containing 1 to 4 carbon atoms.

#### References Cited in the file of this patent

##### UNITED STATES PATENTS

- |           |                       |               |
|-----------|-----------------------|---------------|
| 2,156,724 | Evans et al. -----    | May 2, 1939   |
| 2,271,873 | Perkins et al. -----  | Feb. 3, 1942  |
| 2,339,476 | Hearne et al. -----   | Jan. 18, 1944 |
| 2,605,292 | Shugar et al. -----   | July 29, 1952 |
| 2,658,082 | Urban -----           | Nov. 3, 1953  |
| 2,768,212 | Copenhaver -----      | Oct. 23, 1956 |
| 2,794,029 | Phillips et al. ----- | May 28, 1957  |

##### OTHER REFERENCES

- Gretcher et al.: Jour. Amer. Chem. Soc., vol. 46 (1924), pgs. 1503-04 (2 pages)  
 Palfray et al.: Chem. Abstracts, vol. 22 (1928), pages 4462-63 (2 pages).  
 50 Liston et al.: Jour. Amer. Chem. Soc., vol. 60 (1938), page 1264 (1 page)  
 Hennion et al.: Jour. Organic Chem., vol. 18 (1953), page 1606 (1 page).